# EUROPEAN PATENT SPECIFICATION

(11) **EP 0 033 248 B1**
(45) Date of publication and mention of the grant of the patent: **19.03.1986**
(21) Application number: 81300371.2
(22) Date of filing: 28.01.1981
(51) Int. Cl.: G03G 9/10, G03G 9/00, G03G 19/00

(54) **Magnetic toner and method for developing using same**
Magnetischer Toner und ihn verwendendes Entwicklungsverfahren
Toner magnétique et procédé de développement l'utilisant

(30) Priority: 28.01.1980 US 115974; 28.01.1980 US 115973
(43) Date of publication of application: 05.08.1981
(62) Divisional of application: 84201209.8
(73) Proprietor: XEROX CORPORATION, Rochester New York 14644 (US)
(72) Inventor: Gaudioso, Stephen L., Webster New York (US)
(74) Representative: Weatherald, Keith Baynes

## Description

This invention relates to a single-component magnetic toner.

There has been introduced a magnetic imaging system which employs a latent magnetic image in a magnetizable recording surface, which image may be used in duplicating process, for example, by toning, either once or respectively, transferring the developed image to a suitable support material, such as paper, and fusing the image to said support material.

The latent magnetic image may be provided by any suitable magnetization procedure. Typically, a magnetizable layer of marking material is arranged in imagewise configuration on a magnetic substrate. Well known electrostato- graphic methods are sometimes used to accomplish this. The latent image may then be developed and fused. There a number of known methods for creating the latent image which are described, for example, in US-A-4032923; 4060811, 4074276, 4030105, 4035810, 4101904 and 4121261.

In one such method, the magnetizable toner is developed in imagewise configuration onto an electrophotographic recording surface. The toner is then magnetized, for example, by an electronic recording head. The layer supporting the magnetized toner is then brought into contact with a magnetizable layer and the magnetized toner magnetizes the magnetizable layer in image configuration. A latent magnetic image is thus formed in the magnetizable layer corresponding to the imagewise arrangement of magnetized toner particles.

Concurrently with the growth of interest in magnetic imaging there has been increased interest in magnetic developers to render the latent magnetic images visible. In US-A-3221315 there is described the use of encapsulated ferrofluids in a magnetic recording medium, wherein the ferrofluid orientation in the presence of a magnetic field exhibits a variable light responsive characteristic. In this situation the magnetic recording medium is self-developing in the sense that magnetic marking material need not be employed to render a visible image. In other situations latent magnetic images are rendered visible by magnetic marking material. Thus, for example, in US-A-3627682, there is disclosed binary toners for developing latent magnetic images, which binary toners include a particulate hard magnetic material and a particulate soft magnetic material in each toner particle. The toner particles include two materials in a binder material In US-A-2826634 there is described the use of iron or iron oxide particles either alone or encapsulated in low melting resin or binders for developing latent magnetic images.

Other patents evidencing the continuing interest in improved magnetic developers include US-A-3520811 which discloses that magnetic particles of chromium dioxide appear to catalyze a surface polymerization or organic air drying film forming vehicles such as those employed in oil base materials in order that a coating of polymerized vehicle is formed around the particle; and US-A-3905841 which teaches the prevention of agglomeration and the formation of homogeneous dispersions of cobalt- phosphorous particles into an organic resin binder by treatment with a solution containing sulfuric acid.

Typical fusing methods used in magnetic imaging that have been described in the prior art include, for example, heating the toner image to cause the resin thereof to at least partially melt and become adhered to the transfer medium followed by application of pressure to the toner, such as use of a heater roller. Solvent or solvent vapor fusing has also been used, wherein the resin component of the toner is partially dissolved.

In order to render magnetic imaging systems more amenable to higher speed-duplicating machines, a non-contact flash fusing system, such as that well known in electrophotographic machines, should be used. Aside from higher process speed, improved reliability, especially for paper handling, and higher copy quality is attained. However, in general, toner materials which function satisfactorily with a hot-pressure roll fuser do not perform satisfactorily with a flash fuser. This is true because of the significantly different process-related rheological criteria between these two systems. For contact pressure roll fusing, one needs a toner with shear--dependent viscosity (i.e., low viscosity at high shear and relatively high viscosity at low shear) and sufficient viscoelasticity to avoid hot set-off to the fuser roll over the fusing temperature interval of interest. On the other hand, for non-contact flash fusing, one desires a toner with a strongly temperature-dependent viscosity and minimal elasticity such that the molten toner will rapidly flow and penetrate the paper fibers at the fusing temperature without benefit of contact induced shear. Specifically, for magnetic imaging systems, where the high pigment loading required for development can have an adverse effect on the desired fusing level of the toner, the toner materials designed for and found most acceptable in roll fusing do not have the desired rheological properties for flash fusing.

In accordance with the present invention, there is provided a single-component magnetic toner material which is as claimed in the appended claims.

The toners of the present invention possess higher agglomeration resistance and penetrate extremely rapidly into paper copy sheets under fusing conditions. The toners produce increased definition of characters; more complete transfer of toner images, greater resistance to film formation on reusable image surfaces. They resist the formation of 'fines' under machine operating conditions, exhibiting high resistance to physical degradation, and they show rapid melting properties.

Suitable esterification processes may be used to form the linear resins of this invention. These are discussed in US-A-3590000.

Any suitable magnetite may be employed. About 40% to about 80% by weight of Mapico Black is preferred, with about 65% Mapico Black being optimum. Also, any suitable pigment or colorant may be included in the toner. These may include, for example, carbon black, nigrosine dye, aniline blue, chalco blue, chrome yellow, ultramarine blue, methylene blue chloride, phthalocyanine blue and mixtures thereof.

The amount of magnetic pigment material ranges from 50 to 75% by weight in order to achieve adequate development and fusing at high speed, as for example, with flash fusing. In such formulations the amount of resin used ranged from 25% to 50% by weight.

Additional additives of various types may be added to or used in conjunction with the toners described herein in order to enhance process performance in one or more aspects. For instance Silanox 101 (fumed silica), zinc stearate or other suitable powder flow agents may be used with the toners to aid development. Certain plasticizers, such as diphenylphthalate, are known to dramatically alter the melt viscosity of the toners and may be used to substantially reduce the energy required to fuse the toners to a substrate such as paper. In addition, surface treatment or blending of the toners with magnetic and or conductive additives, for example, certain metal powders, magnetites or carbon blacks, can be used to impart desirable process characteristics, particularly for development, to the toners of this invention.

The toners of the present invention may be prepared by various known methods such as spray drying. In the spray drying method the appropriate polymer is dissolved in an organic solvent like toluene or chloroform or suitable solvent mixture. The toner colorant and/or pigments are also added to the solvent. Vigorous agitation, such as that obtained by the ball milling processes assists in ensuring good dispersion of the colorant or pigment. The solution is then pumped through the atomizing nozzle while using an inert gas, such as nitrogen, as the atomizing agent. The solvent evaporates during atomization resulting toner varies depending on the size of the nozzle. However, particles of a diameter between 0.1 pm and 100 µm generally are obtained Melt blending or dispersion processes can also be used for preparing the toner compositions of the present invention. This involves melting a powdered form of an appropriate polymeric resin and mixing it with suitable colorants and/or pigments. The resin can be melted by heated rolls, which rollers can be used to stir and blend the resin. After thorough blending, the mixture is cooled and solidified. The solid mass that results is broken into small pieces and subsequently finely ground so as to form free flowing toner particles which range in size of from about 0.1 to about 100 um. Other methods for preparing the toners of the present invention include dispersion polymerization, emulsion polymerization and melt blending/crogenic grinding.

The toners of the present invention may be of any suitable size, although particles ranging in size from 3 pm to 20 11m and preferably from 5 µm to 12 µm fuse particularly well in magnetic imaging systems employing flash fusing. When the particles are too fine, poor development with high background may occur. Optimum results are attained with toner particles ranging in size from 6 to 9 µm.

Toner pile height, that is, the average nominal height of the unfused toner layer in the developed image areas of a magnetic image on an appropriate substrate, such as paper, can be an important parameter in influencing the degree or level of image fix (i.e., image permanence) attained for a given flash fusing energies, toner pile heights of from approximately 3 pm to about 30 pm can be employed, with pile heights from about 5 µm to about 20 um preferred and pile heights from about 7 pm to about 15 pm optimum. In the latter regard, magnetic dipole development is particularly suited to the creation of flash fusible images since the development forces can be controlled to produce extremely uniform toner layers of a given thickness across both line and solid area images.

The magnetic imaging systems are generally known in the arts and are described hereinbefore. The magnetic toners of the present invention can be utilized to develop magnetic latent images and a method of developing magnetic latent images according to the invention is characterised by a magnetic toner as described hereinbefore, the toner particles having a pile height of from 3 to 30 pm, preferably 5 to 20 pm.

The following examples further define and described the magnetic toners according to the present invention and methods of utilizing them to develop latent magnetic images. Parts and percentages are by weight unless otherwise indicated.

### Example I

A toner consisting of 35 parts by weight of a propoxylated bisphenol fumarate resin, a polymeric condensation product of 2,2 bis (4 - hydroxy - isopropoxy - phenyl) - propane and fumaric acid, having a melt index of approximately 10, and 65 parts by weight of the magnetite, Mapico Black, commercially available from the Columbian Chemicals Div. of Cities Service Company, is prepared by conventional milling and jetting techniques. The resulting black toner material has a volume average particle size of about 13.3 µm. The material is subsequently dry blended with about 0.4 percent by weight of a flow agent additive, Silanox 101, commercially available from Cabot Company to produce a free-flowing, magnetic developer.

This toner, when used in a magnetic imaging system for developing magnetic images, produced images of uniform, high optical density and excellent resolution. Excellent fixing of these images is obtained for flash fusing input energies from about 0.74 J/cm² to about 1.00 J/cm² for unfused toner pile heights from about 6 pm to about 12 pm, respectively.

### Example II

A toner is prepared in accordance with Example I, with the exception that the resulting black toner material has a volume average particle size of about 7.1 µm, and substantially similar results to those of Example I are obtained with this toner.

### Example III

The procedure of Example I is repeated with the exception that a propoxylated bisphenol fumarate resin having a melt index of approximately 14 is used (volume average particle size was about 6.35 um), and substantially similar results are obtained when such a toner is used for developing a magnetic image.

### Example IV

The procedure of Example I is repeated with the exception that a propoxylated bisphenol fumarate resin having a melt index of approximately 18 is used (volume average particle size was about 8.5 pm), and substantially similar results were obtained when such a toner was used for developing a magnetic image.

### Example V

The procedure of Example IV is repeated with the exception that a toner consisting of 59 parts by weight of the propoxylated bisphenol fumarate resin, having a melt index of 18, and 41 parts by weight of the Mapico Black magnetite is prepared by conventional milling and jetting. The resulting toner has a volume average particle size of about 8.0 um.

This toner, when used in a magnetic imaging system for developing magnetic images, produces images of uniform, high optical density and excellent resolution. Excellent fixing of these images is obtained for flash fusing input energies from about 0.62 J/cm² to about 1.00 J/cm².

### Example VI

A toner consisting of 35 parts by weight of a propoxylated bisphenol fumarate resin, having a melt index of approximately 10, and 65 parts by weight of the polyhedral magnetite, MO-7029, commercially available from Pigments Division of Pfizer Corporation, is prepared by conventional spray drying techniques from chlorofbrm solution. The resulting black toner material has a volume average particle size of about 12.5 µm. This material is subsequently dry blended with about 0.4 percent by weight of a flow additive, Silanox 101, commercially available from Cabot Company, to produce a free-flowing, magnetic developer.

This toner, when used in a magnetic imaging system, gives results substantially similar to those of Example I.

### Example VII

The procedure V is repeated with the exception that the magnetic pigment used was the acicular magnetite, MO-4431, commercially available from the Pigments Division of Pfizer Corporation.

The toner (volume average particle size was about 13.7 pm), when used in a magnetic imaging system for developing magnetic images, produced images of uniform, high optical density and excellent resolution. Adequate fixing of these images is obtained for flash fusing input energies from about 0.93 J/cm² to about 1.32 J/cm².

### Examples VIII-X

The procedure of Example I is repeated using the following materials:
In Example VIII-a polymeric condensation product of 2,2 bis(4-beta hydroxy ethoxy phenyl)-propane and fumaric acid;
In Example IX-a polymeric condensation product of 2,2 bis (3 - mentyl - 4 - beta - hydroxy ethoxy phenyl)-propane and maleic acid anhydride and
In Example X-polymeric condensation product of 2,2 bis (4 - hydroxy isopropoxy phenyl) propane and itaconic acid.

Each of the above toners, when used in a magnetic imaging system, produces images of uniform, high optical density and excellent resolution.

## Claims

1. A single-component magnetic toner comprised of from 25 to 50 percent by weight of a resin which is a polymeric esterification condensation product of 2,2 bis (4 - hydroxy - isopropoxy - phenyl) - propane and fumaric acid; 2,2 bis (4 - hydroxy - isopropoxy - phenyl) - propane and 2,2-dimethyl fumaric acid 2,2 bis (4 - hydroxy - butoxy - phenyl) - propane and fumaric acid; 2,2 bis (4 - hydroxy - butoxy - phenyl) - propane and 2,2-dimethyl fumaric acid; 2,2 bis (4 - hydroxy - ethoxy phenyl) - propane and fumaric acid, 2,2 bis (3 - methyl - 4 - beta - hydroxyethoxyphenyl) - propane and maleic acid anhydride, or 2,2 bis (4 - hydroxy - isopropoxyphenyl) propane and itaconic acid, and from 75 to 50 percent by weight of magnetite.

2. A magnetic toner as claimed in Claim 1, wherein the magnetite is present in an amount of 65 percent by weight.

3. A magnetic toner as claimed in Claim 1 or 2, including a powder flow agent, such as fumed silica or zinc stearate.

4. A magnetic toner as claimed in any preceding Claim, in which the toner particle diameters range from 3 to 20 µm.

5. A toner as claimed in Claim 4, in which the toner particle diameters range in size from 6 to 9 µm.

## Patentansprüche

1. Magnetischer Einkomponenten-Toner, umfassend 25 bis 50 Gew.-% eines Harzes, das ein polymeres Veresterungs-Kondensationsprodukt ist aus 2,2 - Bis(4 - hydroxy - isopropoxy - phenyl)propan und Fumarsäure; 2,2 - Bis(4 - hydroxy - isopropoxy - phenyl)propan und 2,2 - Dimethyl - fumarsäure; 2,2 - Bis(4 - hydroxy - butoxy - phenyl)propan und Fumarsäure; 2,2 - Bis(4 - hydroxy - butoxy - phenyl)propan und 2,2 - Dimethylfumarsäure; 2,2 - Bis(4 - hydroxy - ethoxy - phenyl)propan und Fumarsäure; 2,2 - Bis(3 - methyl - 4 - beta - hydroxy- ethoxyphenyl)propan und Maleinsäureanhydrid oder 2,2 - Bis(4 - hydroxy - isopropoxy- phenyl)propan und Itaconsäure und 75 bis 50 Gew.-% Magnetit.

2. Magnetischer Toner nach Anspruch 1, wobei der Magnetit in einer Menge von 65 Gew.-% vorliegt.

3. Magnetischer Toner nach Anspruch 1 oder 2, beinhaltend ein Pulverfließmittel, wie Fumed Silica oder Zinkstearat.

4. Magnetischer Toner nach einem der vorangehenden Ansprüche, wobei die Tonerteilchendurchmesser im Bereich von 3 bis 20 um liegen.

5. Toner nach Anspruch 4, wobei die Tonerteilchendurchmesser im Bereich von 6 bis 9 pm liegen.

## Revendications

1. Toner magnétique à un composant constitué de 25 à 50% en poids d'une résine qui est un produit de condensation d'une estérification polymère de 2,2 - bis(4 - hydroxy - isopropoxy - phényl) - propane et d'acide fumarique, de 2,2 - bis(4 - hydroxy - isopropoxy - phényl) - propane et d'acide fumarique de 2,2-diméthyle, de 2,2 - bis(4 - hydroxy - butoxy - phényl) - propane et d'acide fumarique, de 2,2 - bis(4 - hydroxy - butoxy - phényl) - propane et d'acide fumarique de 2,2 - diméthyle; de 2,2 - bis(4 - hydroxy - éthoxy - phényl) - propane et d'acide fumarique, de 2,2 - bis(3 - méthyl - 4 - béta - hydroxyéthoxy - phényl) - propane et d'anhydride d'acide maléique, ou de 2,2 - bis(4 - hydroxy - isopropoxyphényl) - propane et d'acide itaconique et de 75 à 50% en poids de magnétite.

2. Toner magnétique selon la revendication 1, où la magnétite est présente suivant une quantité de 65% en poids.

3. Toner magnétique selon la revendication 1 ou la revendication 2, comprenant un agent d'écoulement en poudre, tel que le verre de silice ou le stéarate de zinc.

4. Toner magnétique selon l'une quelconque des revendications précédentes, dans lequel les diamètres des particules de toner sont compris entre 3 et 20 pm.

5. Toner selon la revendication 4, dans lequel les diamètres des particules de toner sont compris entre 6 et 9 um.
